

1

3,233,023

### SPINNING OF POLYPROPYLENE

Richard William Harold Benson, Harrogate, England, assignor to Imperial Chemical Industries Limited, London, England, a corporation of Great Britain  
No Drawing. Filed Feb. 21, 1963, Ser. No. 260,330  
Claims priority, application Great Britain, Feb. 27, 1962,  
7,636/62  
6 Claims. (Cl. 264—168)

This invention relates to the spinning of polypropylene, in particular to the melt spinning of crystalline stereoregular polypropylene prepared by a low pressure process.

It is known from British specification 810,023 to prepare fibres and filaments from crystalline propylene polymers which are linear and essentially unbranched in character. Crystalline polypropylene consists substantially of macromolecules wherein the asymmetric carbon atoms have, at least for long stretches, the same steric configuration. Crystalline stereoregular polypropylene of this type is now widely known as isotactic polypropylene.

Fibres or filaments spun from isotactic propylene polymers may be utilised in several ways. They may be drawn and used as continuous filament yarns or they may be drawn and cut into short lengths and further processed as staple fibre in which form they may be processed on conventional textile machinery either alone or mixed with other natural or synthetic fibres. Staple fibres may be utilised for producing filling materials of high bulk. It is an essential part of the staple fibre process that a wavy form should be imparted to the fibres to assist their processing on conventional textile machinery, especially when mixed with natural fibres having this wavy or crimped form. The crimping of the fibres also imparts softness and bulk to yarns produced from them, leading to greater warmth in fabrics produced from such yarns. The process of crimping the fibres has hitherto been an additional step included after the drawing stage in staple fibre production. Filaments spun from isotactic polypropylene may be utilised also as textured or bulked filament yarns which are produced by, for example, a false-twisting process after the drawing stage of the filament yarn process.

I have found by conducting the spinning process in such a way that the spun yarn has a birefringence between  $10 \times 10^{-3}$  and  $19 \times 10^{-3}$  and an intrinsic viscosity between 1.0 and 3.0 and then cold-drawing the spun yarn to draw ratios of 1.2 to 4.0, that on relaxation of the yarn it will spontaneously take up a helical form. I have also found that it is preferable to stabilise the helical form by a heat treatment for example by treating the relaxed yarn in air at 140° C. for about twenty minutes.

According to the present invention I provide a process for the production of fibres or filaments of isotactic polypropylene as hereinbefore defined having a helically crimped form characterised in that the crimped form is spontaneously developed by spinning the filaments of isotactic polypropylene at such a temperature and at such a throughput from polymer of an intrinsic viscosity such that the intrinsic viscosity of the spun yarn is in the range 1.0 to 3.0 preferably 1.5 to 2.5 and the birefringence of the spun yarn is between  $10 \times 10^{-3}$  and  $25 \times 10^{-3}$  and then drawing the spun yarn to 1.2 to 4.0 times its original length the stretched yarn thereafter being allowed to relax freely and quickly.

Birefringence, which indicates the degree of orientation of the spun filaments, may be measured by means of a

2

polarising microscope fitted with a suitable compensator. The intrinsic viscosity, which is conveniently measured in solution in decalin at 135° C., has the meaning defined in the standard reference textbooks, for example on page 5 309 of the 1953 edition of "Principles of Polymer Chemistry" by P. J. Flory.

While very satisfactory spontaneous crimping of the polypropylene yarn is obtained by the process hereinbefore described I have found that under certain conditions the spontaneous crimping effect may be brought about without the second stage drawing. In a specific embodiment of this form of my invention I have spun isotactic polypropylene, having an intrinsic viscosity of 3.4, at a temperature of 252° C. and a wind up speed of 15 2,000 feet per minute. The spun yarn produced had a birefringence of  $17 \times 10^{-3}$  and an intrinsic viscosity of 2.25. Upon release of the winding tension the spun yarn developed a helical crimp which, on stabilisation for about 20 minutes at a temperature between 100° C. and 140° C., increased to a level corresponding to 13% crimp as hereinafter defined.

I have found also that some control of the environment of the threadline in the region of maximum drawing by controlled cooling or heating allows a further control of 25 the birefringence of the spun yarn and also of the spontaneous crimping effect obtained on relaxation. It is clear that there exists a value of draw ratio, dependant upon the values chosen for the intrinsic viscosity and birefringence of the spun yarn, which will lead to optimum development of spontaneous crimping. By proper control 30 of these factors it is possible to vary the degree of spontaneous crimping from almost none to very high crimp densities.

In a specific embodiment of my invention I spin isotactic polypropylene having an intrinsic viscosity between 35 about 1.5 and 2.5 at a temperature between 200 and 300° C. and a wind-up speed between 1,000 and 5,000 feet per minute so that the spun filaments have a birefringence between  $15 \times 10^{-3}$  and  $20 \times 10^{-3}$  and an I.V. between 1.2 and 2.5. These filaments are then cold drawn using a 40 draw ratio between 1.2 and 4.0 and upon relaxation of the drawn yarn spontaneous crimping of the filaments took place. Degrees of crimping between about 5 and 50 turns/inch have been attained by this technique.

45 The degree of crimping may be expressed either as the number of turns per inch or as the percentage crimp which is expressed by the relation

$$\frac{L_2 - L_1}{L_2} \times 100$$

where  $L_1$  is the length of the filament with the crimps present  $L_2$  is the length of the same filament when extended just sufficiently to remove the crimps.

55 When a second stage drawing step is used I have found that the temperature of the heated pin, roller or other device whereon drawing takes places, may be varied over a wide range of temperature from about 10° C. to about 140° C. and a spontaneous crimping effect is still obtained on release of the drawing tension. I prefer to use a drawing temperature between about 80° C. and 100° C.

Improved spinning and processing as hereinbefore described may be usefully integrated with the melting/compressing procedure for polypropylene which is the subject of British specification 818,100. A suitable apparatus comprises a screw extruder, from which molten poly-

propylene is supplied to a spinneret via a metering pump. Filtration of molten polymer is desirable both before and after it passes through the metering pump, the temperature of the first filter can, if desired, be well below that of the second filter. With such an apparatus polypropylene of high intrinsic viscosity, for example, 3.0 to 4.0, may be used as starting material and thermally degraded in the melter to give the desired level of intrinsic viscosity in the spun yarn.

To obtain a spun yarn having the hereinbefore specified birefringence and intrinsic viscosity the conditions of spinning are varied to suit the particular isotactic polypropylene used and the degree of spontaneous crimping required. I have found, for example, that starting with polypropylene of intrinsic viscosity between 1.0 and 6.0, suitable spinning conditions are a spinneret temperature between 175° C. and 320° C., preferably 180-290° C. and a wind-up speed between about 1,000 and 4,000 feet per minute.

Crimped fibres or filaments produced according to the process of my invention are very suitable for use in textile applications, especially for preparing carpets, blankets, apparel fabrics or other textile products where the crimped structure leads to such desirable properties as resilience, cohesiveness or bulk of the staple or continuous filament yarns comprising such crimped fibres, either alone or mixed with natural fibres or other synthetic fibres. Because of their enhanced bulk and resilience fibers produced by the process of present invention are particularly suitable for use as filling material in, for example, pillows and cushions.

The examples which follow illustrate but in no way limit our invention.

#### Examples 1-4

Isotactic polypropylene having an intrinsic viscosity (in Decalin at 135° C.) of 3.2 to which 0.4% of a suitable antioxidant and 0.1% of a suitable peptiser (a substance added to promote thermal degradation of polypropylene from a higher to a lower molecular weight) has been added was fed into a screw melter from which the molten polymer was supplied to a metering pump and thence through a filter consisting of 10-20 mesh sand to a two hole spinneret (hole diameter 0.015 inch). The screw melter, metering pump and filter were enclosed in an electrically heated jacket which was maintained at the required spinning temperature. The spun yarns were then cold drawn using a water bath at 90° C. at the required draw ratio and at a draw speed of 200 feet per minute. The drawn yarns were then relaxed quickly by cutting the yarn off the draw bobbin and stabilised by heating in air at 140° C. for twenty minutes.

The table which follows shows the effect of spinning temperature and wind-up speed on the intrinsic viscosity and birefringence of the spun yarn and the effect of draw ratio on the degree of spontaneous crimping obtained.

stage drawing was omitted, the winding tension of the spun yarn was released and the yarn allowed to relax freely at 140° C. to develop the full helical crimping effect.

5 The following table shows the percentage crimp developed in yarns spun under various conditions.

| 10 | Spinning Temperature (° C.) | Wind-up Speed (feet/minute) | Spun Yarn Properties |                                | Percentage Crimp |
|----|-----------------------------|-----------------------------|----------------------|--------------------------------|------------------|
|    |                             |                             | Intrinsic viscosity  | Birefringence $\times 10^{-3}$ |                  |
| 15 | 5-----                      | 250                         | 1,120                | 2.45                           | 19               |
|    | 6-----                      | 255                         | 2,000                | 2.45                           | 16               |
|    | 7-----                      | 265                         | 2,000                | 1.94                           | 15               |
| 20 | 8-----                      | 268                         | 3,000                | 1.95                           | 16               |
|    |                             |                             |                      |                                | 25               |

What I claim is:

- 25 1. A process for the production of crimped filaments of isotactic polypropylene comprising producing isotactic polypropylene filaments having an intrinsic viscosity of between about 1.5 and 2.5 and a birefringence of between about  $10 \times 10^{-3}$  to  $19 \times 10^{-3}$ , said producing step including the steps of melt spinning a polypropylene of intrinsic viscosity between 1.0 and 6.0 at a spinneret temperature between 175° C. and 320° C. to form filaments and winding up the filaments at between about 1000 and 5000 feet per minute, said process further comprising subsequently drawing the filaments at between 10° C. and 140° C. at a draw ratio of between about 1.2 and 4.0 and relaxing the drawn filaments to produce spontaneous crimping.
- 30 2. A process according to claim 1 wherein the spinneret temperature is 240° C. to 260° C., the spun filaments have an intrinsic viscosity of 1.8 to 2.2, the wind-up speed is 1000 to 3500 feet per minute, the birefringence of the filaments is  $15 \times 10^{-3}$  to  $19 \times 10^{-3}$  and the draw ratio is 1.25 to 2.0.
- 35 3. A process according to claim 2 wherein the intrinsic viscosity of the polypropylene being spun is about 3.2 and wherein the drawing is carried out at about 90° C. at a draw speed of about 200 feet per minute.
- 40 4. A process according to claim 1 wherein the relaxed yarn is stabilized by heating to a temperature of 100° C. to 140° C.
- 45 5. A process for the production of crimped filaments of isotactic polypropylene comprising producing isotactic polypropylene filaments having an intrinsic viscosity of between about 1.5 and 2.5 and a birefringence of between about  $15 \times 10^{-3}$  and  $10 \times 10^{-3}$ , said producing step in-

|        | Spinning Temperature (° C.) | Wind-up Speed (feet/minute) | Spun Yarn Properties |                     |                             | Draw Ratio | Percentage Crimp | Turns per Inch |
|--------|-----------------------------|-----------------------------|----------------------|---------------------|-----------------------------|------------|------------------|----------------|
|        |                             |                             | Denier               | Intrinsic Viscosity | Birefringence $\times 10^3$ |            |                  |                |
| 1----- | 240                         | 1,000                       | 54                   | 2.2                 | 17                          | 2.0:1      | 41.6             | 10-15          |
| 2----- | 250                         | 2,000                       | 40                   | 1.9                 | 19                          | 1.33:1     | 36.2             | 10-15          |
| 3----- | 250                         | 2,000                       | 49                   | 1.9                 | 18                          | 2.0:1      | 45.5             | 15-20          |
| 4----- | 260                         | 3,500                       | 29                   | 1.8                 | 15                          | 1.25:1     | 24.2             | 5-10           |

#### Examples 5-8

Isotactic polypropylene having an intrinsic viscosity of 3.4 (in Decalin at 135° C.) was spun with the same equipment as in the preceding examples. The second

75 cluding the steps of melt spinning isotactic polypropylene at 250° C. to 270° C. and winding up the filaments at 1120 to 3000 feet per minute, said process further comprising relaxing the yarn directly after the wind-up step.

6. A process according to claim 5 wherein the relaxed yarn is stabilized by heating to a temperature of 100° C. to 140° C.

**References Cited by the Examiner**

**UNITED STATES PATENTS**

3,093,444 6/1963 Martin ----- 18—54 XR

**FOREIGN PATENTS**

1,297,364 5/1962 France.

827,409 2/1960 Great Britain.  
875,108 8/1961 Great Britain.

5 ALEXANDER H. BRODMERKEL, *Primary Examiner.*

MORRIS LIEBMAN, *Examiner.*

C. B. HAMBURG, K. W. VERNON, A. LEAVITT,  
*Assistant Examiners.*